

# UNITED STATES PATENT OFFICE.

HOWARD F. WIERUM, OF UPPER MONTCLAIR, NEW JERSEY, ASSIGNOR TO THE  
SULPHUR SYNDICATE LIMITED, OF LONDON, ENGLAND, A CORPORATION.

## PROCESS OF DESULFURIZING ORES.

1,182,951.

Specification of Letters Patent. Patented May 16, 1916.

No Drawing.

Application filed December 29, 1914. Serial No. 879,614.

To all whom it may concern:

Be it known that I, HOWARD F. WIERUM, citizen of the United States, residing at Upper Montclair, in the county of Essex 5 and State of New Jersey, have invented certain new and useful Improvements in Processes of Desulfurizing Ores, of which the following is a specification.

This invention relates to a method of 10 operating desulfurizing furnaces, in which such an ore as pyrites, pyrrhotite, or other sulfid ores or mattes, or mixtures thereof are roasted to remove the bulk of the sulfur of said ores or mattes, and to convert the major 15 portion of the metals contained therein into oxids, in such a manner as to prevent the escape of any considerable quantities of oxids of sulfur into the atmosphere, in such a manner as to recover if possible, all or 20 the major part of the sulfur eliminated from the ore, in the form of elemental sulfur.

In carrying out my process any type of roaster, similar to the McDougall, Wedge or Herreshoff or practically any conventional 25 type, may be employed.

In carrying out my invention, I preferably proceed as follows:—The ore is fed, preferably in a continuous manner into the compartment, preferably the uppermost 30 compartment of the furnace in the case of a multiple hearth furnace, and in said compartment I maintain a non-oxidizing atmosphere, for example by the admission of flames of oil or gas, which flames are non- 35 oxidizing, and are not highly reducing. It is preferable to maintain these flames as nearly neutral as possible, but since it is impossible to continuously maintain the flames absolutely neutral, it is advisable to have the 40 flames very slightly reducing. In this zone of the furnace, which may comprise one or more hearths, the ore is subjected to a temperature at which the major portion of the feeble atom of sulfur is distilled off. Without 45 out limiting myself to any particular temperatures, I will state that with ordinary pyrites ore containing copper, a temperature of 750° C. to 900° C. may be employed in this zone. During the passage of the 50 ore through this zone the bulk of the feeble atom of sulfur in the pyrites is driven off.

The ore from which the major portion of the less feeble atom has thus been distilled may be then caused to travel to and through another section or zone of the furnace, in 55 which a highly reducing atmosphere is maintained, and a temperature as high as possible is maintained, without melting or fritting the ore passing through it. In this section of the furnace little or no chemical 60 or physical action is performed on the ore, the function of this section of the furnace, in which the highly reducing hot atmosphere is maintained, by means of strongly reducing flames of oil or gas introduced thereto, 65 is to reduce as much as possible of the sulfur dioxid contained in the gases entering said zone. While the ore is not materially changed in passing through this zone of the furnace, I consider it advisable, in most 70 cases, to allow the ore to pass through this zone. However, with certain kinds of ore, and under certain conditions, I may by-pass the ore around or through this second zone, so that the ore will drop from the first zone 75 (neutral or slightly reducing) to the third zone, hereinafter referred to. The ore is now conducted to a third section or zone of the furnace in which an oxidizing atmosphere is maintained, and a temperature high 80 enough to oxidize the larger portion of, or as much as is desirable of, the sulfur remaining in the ore under treatment. From this third section of the furnace, the ore is discharged as usual into hoppers or cars 85 for subsequent treatment, if desired. The gases formed in this third section of the furnace and which contain  $SO_2$ , are conducted through the second section or zone of the furnace, in which the highly reducing, hot 90 atmosphere is maintained, and are there largely reduced to elemental sulfur, which elemental sulfur then passes to and through the first section of the furnace, in which a non-oxidizing but preferably non-reducing, 95 atmosphere is maintained.

By providing the three distinctly different sections described above, I prevent the elemental sulfur, either that distilled from the raw pyrites or that which is produced from  $SO_2$ , from coming into contact with any 100 strongly reducing gases or particles of car-

bon, and thus prevent the formation of any organic or carbonaceous compounds of sulfur which might otherwise be formed.

The three-step process above referred to is particularly applicable to the treatment of ores in which a large amount of pyrites exists. In the treatment of pyrrhotite or matte or similar material containing no considerable amount of feeble atom, the first zone above referred to could be omitted, and the ore subjected first to the strongly reducing atmosphere, and then to the oxidizing atmosphere, although it is found that the treatment of the ore, even when containing no considerable amount of feeble atom, first by the neutral flames, then by the highly reducing flames, and then by the oxidizing atmosphere gives excellent results.

The gases passing from the oxidizing zone contain considerable amounts of sulfur dioxid, which is reduced in the second or reducing zone. The gases leaving the reducing zone aid in maintaining the slightly reducing or neutral atmosphere in the first zone. The gases leaving the uppermost compartments of the furnace, or the neutral zone may be led off to any suitable device for the recovery of elemental sulfur therefrom.

While I have described the process as being carried out in a multiple hearth furnace, I call attention to the fact that other types of furnaces could be used, *e. g.* a long single hearth furnace, provision being made for dividing it into zones for the carrying out of the successive steps. I now prefer, however, a multiple hearth furnace.

In my copending application, Serial No. 825,403, filed June 17, 1914, I have described and claimed a process of desulfurizing ores, such as pyrites, in which the ore, preferably while being rabbled in the upper compartments of an ore roasting furnace of the multiple shelf type, is subjected to the action of a reducing or non-oxidizing flame, and thereafter the ore is subjected to an oxidizing atmosphere, while at a temperature sufficiently high to convert the sulfur remaining in the ore into the form of sulfur dioxid. In the process of said application, the gases travel in the direction opposite to the travel of the ore.

In another copending application Serial No. 848,997, filed July 3, 1914, I have described a process in which sulfid ore is first heated in a strongly reducing atmosphere, for example in the uppermost compartment or compartments of an ore roasting furnace, preferably of the multiple shelf type, after which the ore is subjected to the action of a substantially neutral (that is to say not strongly reducing and not oxidizing) flame and thereafter the ore is subjected, for example on the lower hearths of said furnace,

to the ordinary roasting operation, while the gases travel in a direction opposite to the direction of travel of the ore under treatment.

The present application is in part a continuation of each of said prior applications.

What I claim is:

1. A process of separating sulfur from metallic sulfids, which consists in first subjecting the ore to a temperature sufficient to distil a larger part of the less stable atom of sulfur present in the raw ore, and in an atmosphere which is non-oxidizing; then passing the ore through another section of the same furnace, in which a highly reducing atmosphere is maintained, and a temperature preferably just under the fusing or melting temperature of the material under treatment; then passing the material through a third section of the furnace, in which an oxidizing atmosphere is maintained, in which third section a greater or less amount of the sulfur remaining in the material under treatment is oxidized and sulfur dioxid, usually with some trioxid, present, and passing the gases and vapors formed throughout these successive steps in a direction opposite to that of the travel of the ore, thus providing means for the reduction of sulfur oxids formed in the third section of the furnace to be reduced to sulfur in their passage through the second section of the furnace, and also means for preventing either the oxidation or combination with carbonaceous matter of the elemental sulfur distilled in the first section of the furnace, as well as the elemental sulfur produced in the second section of the furnace.

2. A process of separating sulfur from metal sulfids which comprises subjecting said sulfids to the action of a non-oxidizing flame, and thereafter subjecting said sulfids, while in a heated state to oxidation, passing the gases produced in said step of oxidation into and through a space wherein said gases are subjected to a reducing atmosphere.

3. A process of separating sulfur from sulfid ore which comprises subjecting said ore to the action of a reducing flame, and thereafter subjecting said ore while in a heated state to oxidation, and drawing off the gases and vapors produced in each of said steps, and mingling said gases and vapors together, within the space wherein the ore is subjected to the reducing flame, whereby the sulfur oxids produced in said oxidation are reduced, at least in part, to elemental sulfur.

4. A process of separating sulfur from metal sulfids which comprises subjecting said sulfids to the action of a reducing flame, in a section of the furnace, and thereafter subjecting the same to an oxidizing

atmosphere in another section of the furnace, at a temperature at which a part at least of the sulfur will oxidize to  $\text{SO}_2$ , passing the gases through the sections in which 5 the successive steps are carried out in a direction opposite to the direction of travel of the sulfids through said compartments.

5. A process of separating sulfur from a sulfid ore which comprises subjecting said 10 ore to a non-oxidizing flame in the absence of large amounts of steam, in which step the major portion of the feeble atom of sulfur is distilled, exposing said ore to a reducing flame after the feeble atom has been 15 distilled, and in the absence of large amounts of steam, and then exposing said ore to an oxidizing flame and in the absence of material quantities of steam, said steps being successively performed upon a 20 traveling stream of ore, passing the gases produced in the later steps, through the compartments in which the earlier steps are carried out, in contact with the reducing flame employed in said second step.

25. 6. A process of separating sulfur from sulfid ores, which comprises agitating said ores while treating the same with a non-oxidizing flame, thereafter subjecting said ores to oxidation, passing the gases produced 30 in each of the stages of the process in a direction contrary to that of the ore under treatment, until said gases come into the influence of a reducing flame.

7. A process of separating sulfur from an 35 ore containing both feeble atom of sulfur and fixed atom of sulfur, which comprises separating at least a portion of said feeble atom by subjecting said ore to a non-oxidizing flame, thereafter subjecting said ore to 40 the action of oxidation, to convert a portion of the fixed atom of sulfur of said ore into an oxid of sulfur, subjecting said oxid of sulfur to the action of a reducing flame to reduce the same to elemental sulfur.

45. 8. The method of operating a desulfurizing furnace, which consists of so controlling the atmosphere in the several parts of such furnace, that any oxid of sulfur formed in one part of the furnace where an oxidizing 50 atmosphere is maintained, is subsequently reduced to elemental sulfur in another part of the same furnace, where a reducing atmosphere is maintained.

9. The method of operating a desulfurizing furnace which consists of distilling the major portion of the less stable atom of sulfur from a sulfid ore, in one portion of such furnace, by means of heat generated by incomplete combustion of any suitable hydrocarbon material, such incomplete combustion resulting in the production and maintenance of a hot non-oxidizing atmosphere in said portion of such furnace, thereafter causing the heated ore from which

the major portion of the less stable atom of 65 sulfur has been distilled and driven off, to travel to another portion of such furnace in which an atmosphere is maintained, rich enough in oxygen to oxidize the major portion of the sulfur remaining in said hot ore 70 to oxid of sulfur, then causing these oxid of sulfur to travel to and through a portion of the furnace in which a hot reducing atmosphere is maintained, so that the said oxid of sulfur will be reduced to elemental 75 sulfur in their passage through the hot reducing atmosphere.

10. A process of desulfurizing ores which comprises subjecting said ores, in a non-oxidizing atmosphere to a temperature at 80 which at least the major portion of the less stable atom of sulfur is distilled from the ore in the form of elemental sulfur, passing the ore thus treated to another part of the furnace and there subjecting the same to the 85 influence of an oxidizing atmosphere, at a temperature at which at least a portion of the remaining sulfur is oxidized to  $\text{SO}_2$ ; passing the gases from the portion of the furnace in which the  $\text{SO}_2$  is produced, into 90 and through a part of the furnace in which a reducing atmosphere is maintained, in order to reduce at least the major portion of the  $\text{SO}_2$  to elemental sulfur.

11. A process of desulfurizing ores which 95 comprises subjecting said ores, to the action of a non-oxidizing atmosphere at a temperature at which the major portion of the less stable atom of sulfur is distilled from the ore in the form of elemental sulfur, passing 100 the ore thus treated into another portion of the furnace and there subjecting the same to the influence of an oxidizing atmosphere at a temperature at which at least a portion of the remaining sulfur is oxidized to  $\text{SO}_2$ ; 105 passing the gases from the portion of the furnace in which the  $\text{SO}_2$  is produced into and through a part of the furnace in which a strongly reducing atmosphere is maintained in order to reduce at least the major 110 portion of the  $\text{SO}_2$  to elemental sulfur.

12. A process of separating sulfur from a metal sulfid, which consists of so controlling the temperature and the reducing or oxidizing qualities of the atmosphere in different parts of the furnace in which the process is carried out, that the sulfid will first be subjected to a temperature of at least 700° C., in a non-oxidizing atmosphere, and later to a roasting temperature in an oxidizing atmosphere, and passing the sulfurous gases from the oxidizing portion of the furnace through a portion of the furnace in which a high temperature and a strongly reducing atmosphere are maintained. 115 120 125

13. A process of separating sulfur from metallic sulfids which comprises first subjecting the ore in a non-oxidizing atmos-

sphere, to a temperature at which the larger part of the less stable atom of sulfur distills in elemental form, then passing the ore around a second section of the furnace in which a highly reducing atmosphere is maintained, at a temperature high enough to reduce oxids of sulfur to the elemental form, then passing the material through a third zone of the furnace in which an oxidizing atmosphere is maintained and in which a part at least of the sulfur remain-

ing in the ore is oxidized to oxids of sulfur, passing the gases formed in said last mentioned step, into and through the section in which the hot highly reducing atmosphere 15 is maintained.

In testimony whereof I affix my signature in presence of two witnesses.

HOWARD F. WIERUM.

Witnesses:

RILEY E. SCOTT,  
A. M. PERKINS.